

## UNITED STATES PATENT OFFICE

2,378,761

## CLEANING OXIDES FROM STEEL

Frank Forsberg, Worcester, Mass., assignor to The American Steel and Wire Company of New Jersey, a corporation of New Jersey

Application October 17, 1941, Serial No. 415,467

3 Claims. (Cl. 204—145)

This invention is a method of electrolytically cleaning oxidized steel.

According to the method, the oxidized steel is immersed in molten sodium nitrate, the electric current being passed through this salt to the steel so as to dissociate the former and thus deposit sodium on the latter. It is to be understood that the direction of the current is considered to be from positive to negative whereby the steel will be the cathode. The sodium nitrate dissociates and deposits sodium on the steel, this sodium reacting with the oxide on the steel so that it is oxidized to sodium peroxide.

When the steel is thus cleaned it may be removed from the salt. Since it will be coated with sodium peroxide there is no danger of it again becoming oxidized. The removal of this peroxide coating may be easily effected by rinsing the steel. The rinsing may also function to cool the steel to a point where there is no danger of oxidation, it being obvious that the removal of the sodium peroxide coating leaves its surfaces unprotected. The steel may then be immersed in cold acid to neutralize any sodium peroxide which might not have been removed by the rinsing. That is to say, the acid used is not heated to temperatures common to ordinary pickling operations since this would cause the steel to absorb hydrogen and become subject to acid brittleness.

A specific example of a method embodying the foregoing principles will now be disclosed with the aid of the accompanying drawing, which schematically shows a set-up for practicing the method. No numerals are applied to the various elements of this set-up for the reason that these are all plainly labeled.

In this particular instance, the steel to be cleaned is in the form of wire, and the reason this wire is oxidized is that it is being led from the wire supply reel through a lead annealer from which it exits at temperatures sufficiently high to cause its surface to absorb oxygen from the atmosphere.

Leaving the lead annealer, the wire enters the bath of fused salt where the electrolytic cleaning is to take place. According to the invention, this salt is sodium nitrate which deposits sodium on the wire when a current is passed through it to the latter. The use of this salt involves a further advantage in that evolutions of nitrogen-oxides take place at the surface of the steel kettle which is the anode. This prevents sludges from sticking to the surface of the steel kettle and makes cleaning of its bottom by scraping a rela-

tively simple proposition. It is to be understood that the fused salt may be contained in a conventional steel kettle.

In order to lower the temperature required to maintain the sodium nitrate molten, a mixture of about 80% of this salt and about 20% of potassium nitrate may be used. This enables the use of temperatures of from 700 to 1000 degrees F. and provides for the usual economies connected with the use of lower temperatures. However, the sodium salt is to be considered as the active agent in the electrolytic cleaning.

The voltages used may range from 6 to 12 volts, 10 volts being considered preferable. The time 15 the wire requires to pass through the salt may vary from 30 to 90 seconds, depending on its state of oxidation.

Oxides on the surface of the wire are removed by the sodium reacting to form sodium peroxide. 20 The oxygen of the atmosphere is prevented from combining with the sodium by the fact that the entire reaction takes place beneath the level of the fused salt.

When the wire leaves the electrolytic cleaner 25 it carries a coating of sodium peroxide which prevents its surface from becoming oxidized or blued, it being understood that this might otherwise occur because of the elevated temperature of the wire resulting from its passage through the 30 molten salt. This coating is removed by the passage of the wire through a water rinse which at the same time lowers the temperature of the wire to a point where oxidation need no longer be feared.

35 From the water rinse the wire goes through a bath of cold hydrochloric acid. Since this acid is cold or at least at no greater than room temperature, there is no danger of it imparting acid brittleness to the wire. The only function of this 40 acid is to neutralize any of the basic sodium peroxide which might accidentally remain on the wire after its passage through the water rinse. From the hydrochloric acid bath the wire passes through another water rinse where the acid is 45 removed, and from there it goes on to other processing equipment for galvanizing, tinning, or other operations.

50 Although the specific example of the invention is in connection with steel in the form of wire, it is to be understood that the invention is equally applicable to the cleaning of sheets and other forms of steel.

Furthermore, although the sodium salt is to be considered as the active agent in the electrolytic cleaning, the potassium salt effectively pro-

duces evolutions of nitrogen-oxides which prevent the sludges from sticking to the surface of the steel kettle. This function is also performed by the nitrites of sodium and potassium. The desired prevention of sludge sticking is, in fact, obtained by any compound that does not interfere with the cleaning action of the sodium salt, and which, in addition, decomposes by the electrolytic action at the surface of the steel kettle, so as to form nitrogen-oxide evolutions. At the same time, this desired effect is critically greater in the case of sodium nitrate. Also, sodium nitrate has the further great advantage that it is much more available and, hence, inexpensive than other usable compounds.

This application is a continuation in part of an application filed July 30, 1936, Serial No. 93,481.

I claim:

1. In the art of electrolytically treating metal in a bath including molten sodium compound, the method comprising the use of a ferrous kettle for the bath and the inclusion of sodium nitrate by the bath in conjunction with passing the current from the kettle through the bath to the metal being treated in the latter, whereby the kettle is the anode, the current causing evolutions of nitrogen-oxides at the surfaces of the kettle contacted by the bath, to prevent sludges from sticking to these surfaces and making cleaning of these surfaces by scraping a relatively simple proposition.

2. In the art of electrolytically treating metal

in a bath including molten sodium compound, the method comprising the use of ferrous kettle for the bath and the inclusion of sodium nitrate by the bath in conjunction with passing the current from the kettle through the bath to the metal being treated in the latter, whereby the kettle is the anode, the current causing evolutions of nitrogen-oxides at the surfaces of the kettle contacted by the bath, to prevent sludges from sticking to these surfaces and making cleaning of these surfaces by scraping a relatively simple proposition, the bath consisting mainly of sodium nitrate and sufficient potassium nitrate to lower the fusing temperature of the bath to a degree permitting economical operation.

3. In the art of electrolytically treating metal in a bath including molten sodium compound, the method comprising the use of a ferrous kettle for the bath and the inclusion of a nitrogen and oxygen containing compound by the bath having the characteristic of evolving nitrogen-oxides at the anode when in an electrolytic circuit, in conjunction with passing the current from the kettle through the bath to the metal being treated in the latter, whereby the kettle is the anode, the current causing evolutions of nitrogen-oxides at the surfaces of the kettle contacted by the bath, to prevent sludges from sticking to these surfaces and making cleaning of these surfaces by scraping a relatively simple proposition.

FRANK FORSBERG.